

## UNITED STATES PATENT OFFICE

ADOLF BECK AND GUSTAV SIEBEL, OF BITTERFIELD, GERMANY, ASSIGNEES TO I. G. FARBEININDUSTRIE AKTIENGESELLSCHAFT, OF FRANKFORT-ON-THE-MAIN, GERMANY, A CORPORATION OF GERMANY

PROCESS OF IMPROVING THE RESISTANCE TO CORROSION OF ARTICLES OF MAGNESIUM AND MAGNESIUM ALLOYS

No Drawing. Application filed January 30, 1929, Serial No. 336,323, and in Germany February 2, 1928.

This invention relates to a process of improving the resistance to corrosion of articles and the like of magnesium and high percentage magnesium alloys containing at least about 80% Mg.

Work-pieces of high percentage magnesium-alloys frequently contain surface impurities which give rise to an accelerated corrosion under certain conditions. Thus, for example, the casting skin formed on the surface of cast parts frequently contains compounds of magnesium which may give rise to local attack by corrosion. Pressed, rolled or otherwise worked up pieces are also superficially covered with a skin in which are embedded particles of iron and decomposed organic compounds resulting from the use of tools and lubricants, the presence of which particles, even if only in traces, increases the action of corroding agents, apparently in consequence of local galvanic action.

Now we have ascertained that the resistance of the said alloys against corrosion may be improved by treating the metal pieces with a boiling aqueous solution of dichromates (containing about 100 grams of  $\text{CrO}_3$  per liter), for an hour or longer. By this treatment an extremely thin transparent coating insoluble in water, containing oxidic chrome compounds and having a yellowish brown hue resembling the color of brass is deposited on the surface of the metal.

The effect of the surface treatment contemplated by the present invention can be improved by etching the metal pieces with dilute nitric acid (for example 10% acid) prior to their treatment with boiling aqueous solutions of dichromates, whereby the metal pieces are freed from various superficially adhering impurities, such as for example those arising when the metal pieces are cast in sand moulds, and the superficial casting skin obtained in such cases is removed.

The herein described process may be applied to work-pieces produced by casting, rolling, die-pressing, pressure-casting or by any other method. By virtue of this improvement of the surface qualities, the resistance of these work-pieces to the corroding effect of aqueous solutions is raised to an

exceptional degree. The modified surface produced by the dichromate treatment, furthermore, exhibits the advantageous property of durably retaining lacquer coatings applied thereto. 55

We claim:

1. The process of improving the resistance to corrosion of articles of magnesium and magnesium alloys containing at least about 8% magnesium, which comprises treating 60 same with a boiling aqueous solution of dichromates for about an hour at least.

2. The process of improving the resistance to corrosion of articles of magnesium and magnesium alloys containing at least about 65 80% magnesium, which comprises treating same with a boiling aqueous solution of dichromates for about an hour at least, said treatment being preceded by a preliminary etching with dilute nitric acid. 70

3. The process of improving the resistance to corrosion of articles of magnesium and magnesium alloys containing at least about 80% magnesium which comprises treating the same with a boiling solution consisting of a 75 water-soluble dichromate and water, said dichromate being present in a quantity corresponding to about 100 grams of  $\text{CrO}_3$  per liter, for about one hour at least, said treatment being preceded by a preliminary etching with an aqueous solution containing about 10% nitric acid. 80

In testimony whereof we have hereunto set our hands.

ADOLF BECK 85  
GUSTAV SIEBEL.

90

95

100